

## UNITED STATES PATENT OFFICE.

CARL SCHMIDT, OF BERLIN-TEGEL, GERMANY, ASSIGNOR OF TWO-THIRDS TO SPAR-  
LAGER G. M. B. H., OF BERLIN, GERMANY, A CORPORATION OF GERMANY, AND  
ONE-THIRD TO MARBURG BROTHERS, INC., OF NEW YORK, N. Y., A CORPORATION  
OF NEW YORK.

## PROCESS OF MANUFACTURING ANTIFRICTION BEARINGS AND COMPOUNDS.

No Drawing.

Application filed April 20, 1921. Serial No. 463,042.

*To all whom it may concern:*

Be it known that I, CARL SCHMIDT, a citizen of Germany, residing at Berlin-Tegel, Germany, have invented certain new and useful Improvements in Processes of Manufacturing Antifriction Bearings and Compounds, of which the following is a specification.

My process utilizes the cementing properties of chlormagnesialye, as well as its wood pulp dissolving properties for the manufacture of a magnesia cement of great sliding ability, suitable for the manufacture of sliding bodies or antifriction bearings, which can be used, if so desired, without lubrication.

Bearings have been recommended to be cut out of soapstone and afterwards heated to a temperature of 800°. Bearings have also been made from talc or mica slate with fibrous material added to it, such mixture being molded while in a paste-like condition.

My invention is different from these known processes because I propose to add to magnesium oxide, wood-pulp which has previously been soaked in tar oil or in some other good lubricant. The wood pulp is preferably used in the form of a fine powder but free from rosin. It is advisable to add to my above mixture a small amount of wood soot. To this is added some chlormagnesialye, and of this mixture the bearings or bodies are formed. In order to further decrease the coefficient of friction of the bearings or bodies formed or molded of the material, the bearings after being completed are submerged in hot water in order to dissolve and extract a surplus of salts and thereby to reduce their hygroscopic qualities. In the following a full description is given how such bearings or bodies are produced.

Five to ten units of weight of wood pulp preferably containing no rosin are thoroughly mixed with ten to fifteen units of weight of tar or mineral oil. It is preferable to add to this mixture .2 to .4 units of weight, more or less, of soot, (preferably wood soot) or at any rate sufficient to get a gray colored mixture. Thereafter add 40 to 60 units of weight of burned magnesia,

magnesium-oxide, (MgO) and gradually reduce the latter mixture to a fine dry powder by rubbing and stamping it. To this dry powder is added 20 to 30 units of weight of chlormagnesialye of about 35° Baumé. The latter mixture is worked until it becomes a stiff paste, which latter is pressed into bearings or slidale bodies, such as, for instance, shaft bearings and thrust bearing boxes, guide blocks, loose pulleys, slide valves, etc. The forming or molding must be completed within about three hours after the paste is ready for use, as it gradually hardens and after that time can not be molded easily.

During the hardening of the composition two chemical processes are simultaneously taking place; (a) the partially breaking up and dissolution of the wood pulp to a colloid like substance and (b) the hydratization and cementation of the magnesium oxide and its intimate composition with the wood pulp, which is undergoing the breaking up or dissolution process.

After the material thus formed has become dry and hard, that is after about twenty-four hours, it is treated with hot water to take from it soluble salts adhering to it.

The essential feature of my process is that the wood-pulp is first soaked with oil, which latter effectively prevents that the chlormagnesialye enters into the wood-pulp, which would have the effect that the wood pulp would be broken up or dissolved too much and would become a thin fluid instead of a paste of high viscosity or a plastic mass. The wood-pulp remains soaked with oil, taking from the magnesia cement its stony character so that sliding surfaces are produced which without oiling, work well for light loads and moderate speeds. If a very small quantity of lubricating oil is used from time to time with such bearings, they work exceptionally well at heavy loads and higher speeds.

It is not necessary to form heavy or thick bearings or bodies of this material but a layer of say 3/16" is sufficient. The boxes or bodies can be made of cast iron or any suitable material. My bearing material can be bored out on machine tools if so desired and

polished. Bearings or slidale bodies made according to my process have the advantage of being cheap and permitting a large saving of lubricating oil. They are of special 5 advantage for power transmission shafts, agricultural implements, signal systems, household machinery, and all kinds of hand operated machinery, and show particular advantages at places and under conditions 10 where oiling at regular intervals is difficult and easily overlooked.

Extensive experiments have proved that as a result of the low co-efficient of friction, it is not necessary to add to my material 15 any metal powder to conduct heat, because very little heat is generated.

Approximate proportions of the various ingredients forming my material have been mentioned herein, but I do not restrict myself 20 to the proportions given.

Having thus described my invention, what I claim and desire to cover by Letters Patent of the United States is:

Claims—

25 1. Process of manufacturing an antifriction bearing composition of a magnesia cement, consisting in mixing magnesiumoxyde (magnesia usta) with wood pulp previously

soaked with oil, and chlormagnesialye, the resulting paste being dried to a cement of 30 great sliding ability.

2. Process of manufacturing an antifriction bearing composition of a magnesia cement, consisting in mixing magnesiumoxyde with wood pulp previously soaked with oil, 35 and chlormagnesialye, the resulting paste being dried to a cement of great sliding ability and then washed with hot water.

3. Process of manufacturing antifriction bearings of magnesia cement, characterized 40 by the fact that magnesiumoxyde is mixed with wood pulp previously soaked with oil, and chlormagnesialye, the resulting paste being formed and then dried to bodies of great sliding ability.

4. Process of manufacturing antifriction bearings of a magnesia cement, characterized by the fact that magnesiumoxyde is mixed with wood pulp previously soaked with oil, 50 and chlormagnesialye, the resulting paste being formed or molded to bodies, dried and then washed with hot water.

In testimony that I claim the foregoing as my invention I have signed my name to this specification.

CARL SCHMIDT.